

# UNITED STATES PATENT OFFICE.

GEORGE H. CHARLS, OF CANTON, OHIO.

## METHOD OF ENHANCING RUST-RESISTING QUALITIES OF IRON.

1,355,590.

Specification of Letters Patent. Patented Oct. 12, 1920.

No Drawing.

Application filed April 7, 1920. Serial No. 371,882.

To all whom it may concern:

Be it known that I, GEORGE H. CHARLS, a citizen of the United States, and a resident of Canton, Stark county, State of Ohio, have invented an Improvement in Methods of Enhancing Rust-Resisting Qualities of Iron, of which the following is a specification.

This invention relates to methods of enhancing the rust-resisting qualities of iron. One of the objects thereof is to provide a practical and reliable art for achieving the above result. Another object is to provide an art of the above nature which may be readily carried on at low cost. Other objects will be in part obvious and in part pointed out hereinafter.

The invention accordingly consists in the features of the art hereinafter illustratively described and as set forth in the following claims.

In carrying on this process the iron is placed in molten form; and it may here be noted that the term "iron" is broadly used even though it might contain a small amount of carbon and thus include what might more literally be termed "steel." It is also to be noted that with the iron may be included such elements as sulfur and phosphorus in small quantities which are commonly found in commercial iron.

To the iron in this molten form is added a small amount of molybdenum which may be in the form of molten ferro-molybdenum. This may be added in the furnace, ladle, or even in the ingot, and permeates the entire mass.

It is to be noted that the amount of molybdenum added is small, preferably not exceeding .50%, and for best results being in the neighborhood of .15% or even lower. The molybdenum however should not be less than the sulfur content. Also the carbon should be maintained low, and if it is present in the molten iron to an amount exceeding .20%, it should be reduced. The resultant compound should for best results contain not more than .10% of carbon. When the ingot has solidified, it is formed into the desired shape, being especially adapted for rolling into sheets.

By this addition of a small amount of molybdenum and the maintenance of the

carbon at a low value, the resultant metal is given in a marked degree the ability to resist rust without heat treatment or treatment of its surface. The addition of the molybdenum, moreover, in small quantities, is of value even with the iron without carbon present; excellent results having been found in this method of treatment of metal from which the carbon has been entirely eliminated.

As certain variations might be made in the above art, it is to be understood that the matter herein set forth is in certain respects illustrative.

I claim as my invention:—

1. The herein described art of enhancing the rust-resisting qualities of iron which consists in adding thereto with the metal in molten form, amount of molybdenum less than one per cent.

2. The herein described art of enhancing the rust-resisting qualities of iron which consists in adding thereto with the metal in molten form, a small amount of molybdenum, and keeping the carbon content below .20%.

3. The herein described art of enhancing the rust-resisting qualities of iron which consists in preparing a small amount of molten metal containing molybdenum, preparing iron in molten form with the carbon below .20%, adding the molybdenum-containing metal to the iron, and permitting the resultant alloy to cool.

4. The herein described art of enhancing the rust-resisting qualities of iron which consists in preparing a small amount of molten metal containing molybdenum, preparing iron in molten form with the carbon below .20%, adding the molybdenum-containing metal to the iron, and permitting the resultant alloy to cool, the molybdenum being added in such proportion as to give less than .20% thereof in the final alloy.

5. The herein described art of enhancing the rust-resisting qualities of iron which consists in adding thereto an amount of molybdenum less than .20% and keeping the carbon content below .20%.

In testimony whereof I have signed my name to this specification this 3rd day of March, 1920.

GEORGE H. CHARLS.